

Feb. 26, 1929.

1,703,470

H. BRADSHAW

PHOTOGRAPHIC FILM

Filed March 4, 1927



Fig. 1



Fig. 2



Fig. 3



Fig. 4

H. Bradshaw Inventor

By his attorney

*Edward E. Thompson*

Patented Feb. 26, 1929.

1,703,470

# UNITED STATES PATENT OFFICE.

HAMILTON BRADSHAW, OF WILMINGTON, DELAWARE, ASSIGNOR TO E. I. DU PONT DE NEMOURS & COMPANY, OF WILMINGTON, DELAWARE, A CORPORATION OF DELAWARE.

## PHOTOGRAPHIC FILM.

Application filed March 4, 1927. Serial No. 172,924.

This invention relates to photographic film of the so-called "non-static" type. In the motion picture art, for example, trouble is experienced with static electrical charges on the film, which are generated during manufacture, and are especially objectionable when generated after the application of the sensitive coating when the film comes in contact with rollers, and which are also generated when the film is run through cinematographic apparatus. These charges, if not counteracted, cause markings on the film. The present invention has to do with a film which by virtue of its construction, overcomes or eliminates "static" difficulties of the character mentioned. The object of this invention is to provide a film having the mentioned and other desirable characteristics.

For several reasons which are well understood, it is desirable that the film base or support should be primarily of cellulose nitrate. A difficulty of this material is, however, that it strongly charges electrically, charging negatively. (The gelatine-silver halid emulsion layer charges positively.) In accordance with the present invention there is applied to the back of the film support, i. e. the side opposite that carrying the emulsion, a layer, desirably in the character of a thin backing, comprising a derivative of cellulose which charges either positively or at least much less negatively than cellulose nitrate. Thus a film is obtained which, while mainly cellulose nitrate, as is desirable, is yet non-static to a substantial degree. Whether it be made up to be completely non-static, or but nearly so, will depend, of course, on the desire in any particular case. In particular conformity with the invention, the backing may desirably comprise a cellulose carbamate, conveniently a urethane derivative of cellulose, such as cellulose phenylurethane or cellulose methylurethane.

Without restricting the invention thereto, films embodying the same are illustrated in the accompanying drawing. In the drawing, the figures are exaggerated conventional cross-sectional views, specific description of each figure being evidently unnecessary in view of the legends thereon.

When carrying a sensitized emulsion, a film exemplifying the present invention preferably comprises a central layer of cellulose nitrate with a sensitized emulsion layer on the one side and a thin layer comprising a cel-

lulose urethane on the other. Plainly, the backing may, if desired, comprise more than one cellulosic derivative, so that the cellulose carbamate may be mixed with other cellulosic derivatives such as, for example, cellulose nitrate or acetate.

The general methods of casting a film body and of applying a backing to it are well known in the art and need not be described here in detail; but as illustrating the invention, without however, confining it to the examples given, the following formulas are given:

1. A dope suitable for casting a film to which emulsion, and backings of the present invention, may be applied, cellulose nitrate 15 parts by weight, acetone 70 parts, camphor 2, ethyl alcohol 10 and amyl alcohol 2 parts.

### 2. Backing solutions

(a) 1 part cellulose phenylurethane, 19 75 parts acetone, 80 parts ethyl alcohol.

(b) 1 part cellulose phenylurethane, 1 part cellulose acetate, 23 parts acetone and 75 parts ethyl alcohol.

(c)  $\frac{1}{2}$  part cellulose phenylurethane,  $\frac{1}{2}$  80 part cellulose methylurethane and 24 parts acetone and 75 parts ethyl alcohol.

Cellulose nitrate may be used in the backing solutions; for example, in "b", a like number of parts of the nitrate may be substituted 85 for the acetate, but I prefer the acetate. In Figures 2, 4 and 3 are illustrated films having backings provided by solutions such as a, b and c, respectively, while Figures 1 and 4 illustrate the use of "another cellulose derivative" (Fig. 1). e. g. the nitrate or acetate (Fig. 4).

All backings are applied as a solution, as will be plain to those skilled in the art (conveniently by means of a roller dipping in a 95 trough) and the solvents evaporated. The backing layer may be very thin, and it has no effect upon the emulsion when the film is rolled. As indicated, the carbamate used is soluble, to a substantial extent, in desirable 100 solvents.

The terms "positive" and "negative" are used to denote that the materials mentioned will develop a positive or negative charge when acted on frictionally. The extent to 105 which the film is completely non-static, depends on various conditions; but, in any case the employment of layer on the back side of the cellulose nitrate, which is either positive (like the emulsion) or less strongly negative 110

than ordinary cellulose nitrate, e. g. the cellulose nitrate used as the body layer, is highly advantageous. In my broad claims I use "carbamate" generically, to include both unsubstituted and substituted carbamates.

5 I claim:

1. A photographic film, including a body layer comprising a negative material, and a layer comprising a carbamate of cellulose.
- 10 2. A photographic film, including a body layer comprising a negative material, and a layer comprising a substituted carbamate of cellulose.
- 15 3. A photographic film, including a body layer of cellulose nitrate, and a layer comprising a carbamate of cellulose.
4. A photographic film, including a body

layer of a negative material, and a layer comprising a cellulose carbamate together with another derivative of cellulose.

20

5. A photographic film having a layer comprising a cellulose ester having the group



25

in which R may be hydrogen, an alkyl, or an aromatic, radical.

6. A photographic film comprising a cellulose nitrate body layer carrying on the one side a positive emulsion and on the other side 30 a backing comprising cellulose phenylcarbamate.

In testimony whereof I affix my signature.

HAMILTON BRADSHAW.